# EUROPEAN PATENT SPECIFICATION

(11) **EP 2 028 256 B1**
(45) Date of publication and mention of the grant of the patent: **28.08.2019**
(21) Application number: 08104153.5
(22) Date of filing: 29.05.2008
(51) Int. Cl.: C10M 169/04, C10M 141/10, C10N 40/04, C10N 30/06

(54) **Lubricating oils having improved friction stability**
Schmieröle mit verbesserter Reibungsstabilität
Huiles de lubrification disposant d'une stabilité de friction améliorée

(30) Priority: 29.06.2007 US 770966
(43) Date of publication of application: 25.02.2009
(73) Proprietor: Infineum International Limited, Abingdon Oxfordshire OX13 6BB (GB)
(72) Inventor: Cogen, Kerry Lynn, c/o Infineum USA L.P., Linden, New Jersey 07036 (US); Gorda, Keith R., c/o Infineum USA L.P., Linden, New Jersey 07036 (US); Noles Jr., Joe R., c/o Infineum USA L.P., Linden, New Jersey 07036 (US); Watts, Raymond F., c/o Infineum USA L.P., Linden, New Jersey 07036 (US)
(74) Representative: Hart, Richard Joseph

(56) References cited:
- EP-A1- 1 645 616
- WO-A1-97/14773
- WO-A1-99/11743
- US-A1- 2003 220 206

## Description

This invention relates to a lubricating oil composition having excellent friction stability, particularly power transmitting fluids such as automatic transmission fluids (hereinafter referred to as "ATFs"), continuously variable transmission fluids ("CVTFs"), and double clutch transmission fluids ("DCTFs"), and more particularly having excellent frictional characteristics during high speed clutch engagements.

The transmissions to which this invention is applicable are those transmissions that contain a lubricated wet clutch that is used under conditions of high energy dissipation. These types of applications include the clutches in an automatic transmission used to accomplish ratio or speed changes; wet starting clutches in automatic, continuously variable or double clutch transmissions; or clutches used in torque vectoring or interaxle differential applications. These clutches can be characterized as having high differential speed between the two members of the clutch and high energy dissipation in the "engagement" or "lock up" of the clutch.

A common goal of automobile builders is to produce vehicles that are more durable and perform more reliably over their service life. One aspect of increased durability and reliability is to produce vehicles that need a minimum of repairs during their service life. A second aspect is to have vehicles that perform consistently throughout this "lifetime". In the case of automatic transmissions, not only should the transmission not fail during the lifetime of the vehicle, but its shift characteristics should not perceptibly change over this period. Since shift characteristics of automatic transmissions are heavily dependent on the frictional characteristics of the ATF, the fluid needs to have very stable frictional performance with time, and therefore mileage. This aspect of ATF performance is known as friction stability. Currently many vehicle builders are moving to "fill-for-life" automatic transmission fluids; this trend further increases the need for friction stability of the ATF, since the fluid will no longer be replaced at 15,000 to 50,000 mile service intervals.

A common method for determining the friction durability of an ATF is through the use of an SAE #2 friction test machine. This machine simulates the high speed engagement of a clutch by using the clutch as a brake, thereby absorbing a specified amount of energy. The energy of the system is chosen to be equivalent to the energy absorbed by the clutch in completing one shift in the actual vehicle application. The machine uses a specified engagement speed, normally 3600 rpm, and a calculated inertia to provide the required amount of energy to the test clutch and fluid. The clutch is lubricated by the fluid being evaluated, and each deceleration (i.e., braking) of the system is termed one cycle. To evaluate friction stability many cycles are run consecutively. Increasing emphasis on friction stability by original equipment manufacturers (OEMs) has caused the total number of cycles required to demonstrate satisfactory friction durability to increase from several hundred in the 1980's to 10,000 or more in some current specifications. For example see the Ford MERCON® V Automatic Transmission Fluid for Service specification.

There are two methods of assessing improved friction durability. One is to maintain certain friction characteristics over a longer period of time (i.e. over more cycles). The second is to allow less change in each friction parameter over the course of the same number of cycles. Both methods provide indications that the vehicle shift characteristics will be consistent over a longer number of miles.

Friction control in a power transmission fluid such as an ATF, CVTF or DCTF is primarily the function of the friction modifiers in the fluid. However, the thermal and oxidative stresses under which such fluids are used in the transmissions lead to additive degradation and thereby changes in fluid properties. Oxidation or thermal destruction of the friction modifiers is often first seen in the fluid as rising static friction. Rising static friction causes abrupt shifts which vehicle occupants can feel as a jerk or lurch as the shift completes. Rising static friction is a common mode of failure of power transmission fluids. In some circumstances, however, oxidation of friction modifiers can transform them into more active species. In these situations static friction can actually decrease during service. Lowering of static friction, while not normally an issue for the vehicle occupant, can lower the holding capacity of the clutches in the transmission. Lowering of holding capacity can cause the clutches to slip under high loads, e.g. towing or rapid acceleration, making them prone to overheat and ultimately to fail. Therefore the best power transmission fluids have extremely stable static friction levels that are well maintained with use.

Conventionally, there are two ways to improve friction stability of a power transmission fluid. One way is to increase the amount of friction modifier in the fluid. This has the desired effect of improving friction stability, by providing a higher reservoir of friction modifier in the oil, but increasing the amount of friction modifier has the undesirable secondary effect of lowering the friction coefficients of the fluid to undesirable levels, especially the static coefficient of friction. The second way is to improve the oxidation resistance of the fluid, through the concurrent use of oxidation inhibitor additives, particularly to reduce the generation of polar products of oxidation which thereafter compete with the friction modifiers for the friction surface. Reducing fluid oxidation therefore has the potential to improve long term control of friction.

U.S patents 5,750,476 and 5,840,662 report that a combination of antioxidants, oil soluble phosphorus compounds, and specific low potency friction modifiers can confer outstanding friction durability to ATFs. These low potency friction modifiers are characterized by the fact that once a saturation concentration of the friction modifier is reached in the fluid, increasing the concentration causes no further reduction in the measured friction levels. Fluids can thus be treated with very high concentrations of these low potency friction modifiers to create a larger reservoir of additive in the oil and still exhibit satisfactory levels of friction. It is believed that as the low potency friction modifier molecules are consumed, through shearing or oxidation, there is always an ample concentration available to take their place on the friction surfaces. An oil-soluble phosphorus-containing compound must also be present to protect the system from wear.

However, such solutions by definition demand the use of high quantities of additive. A need exists for solutions which make more efficient use of chemical resources and are more cost effective.

Similarly, the additional requirement for oxidation inhibitors leads to more complex formulations, and the prospect of greater development and usage costs.

We have now found that greater thermal and oxidative stability can be conferred on one class of friction modifier, namely a polyalkylene polyamine based friction modifiers, without any loss of its ability to control friction, by the acylation of at least one secondary amino group present in its polyamine moiety. Where more than one secondary amino group is present in the polyamine chain, particularly good stability can be achieved by acylating a plurality, and preferably all, of the secondary amino groups present in the friction modifier.

Such friction modifiers show improved properties over existing solutions and provide a more cost-effective solution to the problem of friction durability in oils, especially in power transmission fluids.

US2003220206 discloses a lubricant composition which comprises a lubricant base oil and one or more compounds resulting from the modification of a specific succinimide, with one or more compounds selected from the group consisting of carboxylic acids and derivatives thereof, sulfuric compounds and triazoles. The composition is used for automatic transmissions and/or continuously variable transmissions.

WO97/14773 A1 describes lubricating compositions containing a reaction product of a maleated bis(iso-octadecenyl succinimide) and TEPA. The compositions are said to be suitable as automatic transmission fluids.

WO 99/11743 A1 describes lubricating compositions which contain an amine-containing friction modifier and an oil-soluble phosphorus : compound. The compositions are said to provide good friction stability.

In a first aspect, this invention relates to a lubricating oil composition comprising a base lubricating oil, at least one oil soluble thioalkyl phosphite ester compound in an amount delivering from 5 to 5000 ppm of phosphorus into the oil and at least one polyalkylene polyamine-based friction modifier having the structure: In an amount of 0.1 to 10 weight percent in the composition.

In another aspect, the invention relates to the use of the composition of the first aspect in a power transmission.

### DETAILED DESCRIPTION OF THE INVENTION

This invention concerns a method for improving the friction stability of lubricating oils, without disadvantageously lowering the coefficients of friction. It comprises the combined use in the oil of a friction modifier derived from a defined polyalkylene polyamine and an oil-soluble source of phosphorus. This combination of additives provides outstanding friction stability to lubricating oils, especially transmission fluids.

While the benefits of this invention are contemplated to be applicable to a wide variety of lubricating oils wherein friction modifiers are usefully employed (e.g., crankcase engine oils, etc.), particularly preferred compositions are power transmitting fluids, especially automatic transmission fluids (ATFs), continuously variable transmission fluids (CVTFs) and double clutch transmission fluids (DCTFs). Examples of other, less preferred types of power transmitting fluids included within the scope of this invention are gear oils, hydraulic fluids, tractor fluids, universal tractor fluids and the like. These power transmitting fluids can be formulated with a variety of additional performance additives and in a variety of base oils.

### The Polyalkylene Polyamine-based Friction Modifier used in the invention

The friction modifier used in the invention has the structure : which may suitably by formed by the acetylation of the reaction product of diethylene triamine and the requisite isomerised octadecenyl succinic anhydride. This material has been found to give especially good performance in the present invention.

The treat rate of the friction modifier is from 0.1 to 10, preferably 0.5 to 7, and most preferably from 1.0 to 5.0 weight percent in the lubricating oil composition.

Examples of the preparation of typical friction modifier materials of the invention are given below. These examples are intended for illustration, and the invention is not limited to the specific details set forth in the examples.

### PREPARATIVE EXAMPLES

Example A (Preparation of isomerised succinimide) - Into a one liter round bottomed flask fitted with a mechanical stirrer, nitrogen sweep, Dean Starke trap and condenser was placed 352 gm (1.00 mole) of iso-octadecenylsuccinic anhydride (ODSA from Dixie Chemical Co.). A slow nitrogen sweep was begun, the stirrer started and the material heated to 130°C.Immediately thereafter, 95 gm (0.50 moles) of commercial tetraethylene pentamine was added slowly via an addition funnel to the hot stirred iso-octadecenylsuccinic anhydride. The temperature of the mixture was increased to 150°C where it was held for two hours. During this heating period 10 ml. of water (-50% of theoretical yield) were collected in the Dean Starke trap. The flask was cooled to yield the product. Yield: 435 gm. Percent nitrogen: 8.1.
Example B (Preparation of the isomerised succinimide) - The same procedure was followed as in Example A, except that the following amounts were used: iso-octadecenylsuccinic anhydride, 700 gm (2.0 moles), and diethylenetriamine, 103 gm (1.0 mole). The water recovered was 32 ml. Yield: 765 gm. Percent nitrogen: 5.5.
Example C (Preparation of the acylated isomerised succinimide of the invention) Into a one liter round bottomed flask fitted with a mechanical stirrer, nitrogen sweep, Dean Starke trap and condenser was placed 765 gm (1.0 mole) of the product of Example B. A slow nitrogen sweep was begun, the stirrer started and the material heated to 90°C. Acetic anhydride, 102 gm (1.0 mole) was added drop wise through an addition funnel. Once the addition was complete the temperature was raised to 140°C and held for 3 hours. Residual acetic acid was removed by distillation at 150°C at 50 mm Hg. Yield: 805 gm. Percent nitrogen: 5.2.
Example D (Preparation -of the acylated isomerised succinimide not according the invention) - The same procedure was followed as in Example C, except that the following amounts were used: Product of Example B, 765 gm (1.0 mole); caprolactone 131 gm (1.15 moles). The mixture was heated at 170°C for 6 hours followed by the addition of 2 mls of stannous octanoate. After addition of the octanoate the temperature was increased to 180°C for an additional 4 hours. Yield: 895 gm. Percent nitrogen: 4.7
Example E (Preparation of the acylated isomerised succinimide not according the invention) - Into a one liter round bottomed flask fitted with a mechanical stirrer, nitrogen sweep, Dean Starke trap and condenser was placed 429 gm (0.50 moles) of the product of Example A. A slow nitrogen sweep was begun, the stirrer started and the material heated to 90°C. Acetic anhydride, 61 gm (0.5 moles) was added drop wise through an addition funnel. Once the addition was complete the temperature was raised to 140°C and held for 3 hours. Residual acetic acid was removed by distillation at 150°C at 50 mm Hg. Yield: 485 gm. Percent nitrogen: 7.1.

A preferred oil soluble thioalkyl phosphite ester compound, for example is as produced in U.S. 5,314,633. The most preferred compounds are as illustrated by Example G below.

The thioalkyl phosphite ester compound delivers from 5 to 5000 ppm phosphorus into the oil. A preferred concentration range is from about 10 to about 1000 ppm of phosphorus in the finished oil and the most preferred concentration range is from about 50 to about 500 ppm.

### EXAMPLE

EXAMPLE G - An alkyl phosphite mixture was prepared by placing in a round bottom 4-neck flask equipped with a reflux condenser, a stirrer and a nitrogen bubbler, 194 grams (1.0 mole) of dibutyl hydrogen phosphite. The flask was flushed with nitrogen, sealed and the stirrer started. The dibutyl hydrogen phosphite was heated to 150°C under vacuum (-90 kPa) and 190 grams (1 mole) of hydroxylethyl-n-octyl sulfide was added through a dropping funnel over about one hour. During the addition approximately 35 ml of butanol was recovered in a chilled trap. Heating was continued for about one hour after the addition of the hydroxylethyl-n-octyl sulfide was completed, no additional butanol was evolved. The reaction mixture was cooled and analyzed for phosphorus and sulfur. The final product had a TAN of 115 and contained 8.4% phosphorus and 9.1% sulfur.

Other additives known in the art may be added to the lubricating oil of the invention, or included in the additive composition of the invention. These additives include dispersants, antiwear agents, corrosion inhibitors, detergents, extreme pressure additives, and the like. They are typically disclosed in, for example, "Lubricant Additives" by C. V. Smallheer and R. Kennedy Smith, 1967, pp. 1-11 and U.S. Patent 4,105,571.

Representative amounts of these additives in an ATF are summarized as follows:

| additive | (Broad) Wt.% | (Preferred) Wt.% |
|---|---|---|
| VI Improvers | 1 - 12 | 1 - 4 |
| Corrosion Inhibitor | 0.01 - 3 | 0.02 - 1 |
| Dispersants | 0.10 - 10 | 2 - 5 |
| Antifoaming Agents | 0.001 - 5 | 0.001 - 0.5 |
| Detergents | 0.01 - 6 | 0.01 - 3 |
| Antiwear Agents | 0.001 - 5 | 0.2 - 3 |
| Pour Point Depressants | 0.01 - 2 | 0.01 - 1.5 |
| Seal Swellants | 0.1 - 8 | 0.5 - 5 |
| Lubricating Oil | Balance | Balance |

Suitable dispersants include long chain (i.e. greater than forty carbon atoms) substituted hydrocarbyl succinimides and hydrocarbyl succinamides, mixed ester/amides of long chain (i.e. greater than forty carbon atoms) hydrocarbyl-substituted succinic acid, hydroxyesters of such hydrocarbyl-substituted succinic acid, and Mannich condensation products of long chain (i.e. greater than forty carbon atoms) hydrocarbyl-substituted phenols, formaldehyde and polyamines. Mixtures of such dispersants can also be used.

The preferred dispersants are the long chain alkenyl succinimides. These include acyclic hydrocarbyl substituted succinimides formed with various amines or amine derivatives such as are widely disclosed in the patent literature. Use of alkenyl succinimides which have been treated with an inorganic acid of phosphorus (or an anhydride thereof) and a boronating agent are also suitable for use in the compositions of this invention as they are much more compatible with elastomeric seals made from such substances as fluoro-elastomers and silicon-containing elastomers. Polyisobutenyl succinimides formed from polyisobutenyl succinic anhydride and an alkylene polyamine such as triethylene tetramine or tetraethylene pentamine wherein the polyisobutenyl substituent is derived from polyisobutene having a number average molecular weight in the range of 500 to 5000 (preferably 800 to 2500) are particularly suitable. Dispersants may be post-treated with many reagents known to those skilled in the art. (see, e.g., U.S. Pat. Nos. 3,254,025, 3,502,677 and 4,857,214).

The additive combinations of this invention may be combined with other desired lubricating oil additives to form a concentrate. Typically the active ingredient (a.i.) level of the concentrate will range from 20 to 90%, preferably from 25 to 80%, most preferably from 35 to 75 weight percent of the concentrate. The balance of the concentrate is a diluent typically comprised of a lubricating oil or solvent.

Lubricating oils useful in this invention are derived from natural lubricating oils, synthetic lubricating oils, and mixtures thereof. In general, both the natural and synthetic lubricating oil will each have a kinematic viscosity ranging from about 1 to about 100 mm²/s (cSt) at 100°C, although typical applications will require each oil to have a viscosity ranging from about 2 to about 8 mm²/s (cSt) at 100°C.

Natural lubricating oils include animal oils, vegetable oils (e.g., castor oil and lard oil), petroleum oils, mineral oils, and oils derived from coal or shale. The preferred natural lubricating oil is mineral oil.

Suitable mineral oils include all common mineral oil basestocks. This includes oils that are naphthenic or paraffinic in chemical structure. Oils that are refined by conventional methodology using acid, alkali, and clay or other agents such as aluminum chloride, or they may be extracted oils produced, for example, by solvent extraction with solvents such as phenol, sulfur dioxide, furfural, dichlordiethyl ether, etc. They may be hydrotreated or hydrofined, dewaxed by chilling or catalytic dewaxing processes, or hydrocracked. The mineral oil may be produced from natural crude sources or be composed of isomerized wax materials or residues of other refining processes.

Typically the mineral oils will have kinematic viscosities of from 2.0 mm²/s (cSt) to 8.0 mm²/s (cSt) at 100°C. The preferred mineral oils have kinematic viscosities of from 2 to 6 mm²/s (cSt), and most preferred are those mineral oils with viscosities of 3 to 5 mm²/s (cSt) at 100°C.

Synthetic lubricating oils include hydrocarbon oils and halo-substituted hydrocarbon oils such as oligomerized, polymerized, and interpolymerized olefins [e.g., polybutylenes, polypropylenes, propylene, isobutylene copolymers, chlorinated polylactenes, poly(1-hexenes), poly(1-octenes), poly-(1-decenes), etc., and mixtures thereof]; alkylbenzenes [e.g., dodecyl-benzenes, tetradecylbenzenes, dinonyl-benzenes, di(2-ethylhexyl)benzene, etc.]; polyphenyls [e.g., biphenyls, terphenyls, alkylated polyphenyls, etc.]; and alkylated diphenyl ethers, alkylated diphenyl sulfides, as well as their derivatives, analogs, and homologs thereof, and the like. The preferred oils from this class of synthetic oils are oligomers of α-olefins, particularly oligomers of 1-decene.

Synthetic lubricating oils also include alkylene oxide polymers, interpolymers, copolymers, and derivatives thereof where the terminal hydroxyl groups have been modified by esterification, etherification, etc. This class of synthetic oils is exemplified by: polyoxyalkylene polymers prepared by polymerization of ethylene oxide or propylene oxide; the alkyl and aryl ethers of these polyoxyalkylene polymers (e.g., methyl-polyisopropylene glycol ether having an average molecular weight of 1000, diphenyl ether of polypropylene glycol having a molecular weight of 1000 - 1500); and mono- and poly-carboxylic esters thereof (e.g., the acetic acid esters, mixed C₃-C₈ fatty acid esters, and C₁₂ oxo acid diester of tetraethylene glycol).

Another suitable class of synthetic lubricating oils comprises the esters of dicarboxylic acids (e.g., phthalic acid, succinic acid, alkyl succinic acids and alkenyl succinic acids, maleic acid, azelaic acid, suberic acid, sebasic acid, fumaric acid, adipic acid, linoleic acid dimer, malonic acid, alkylmalonic acids, alkenyl malonic acids, etc.) with a variety of alcohols (e.g., butyl alcohol, hexyl alcohol, dodecyl alcohol, 2-ethylhexyl alcohol, ethylene glycol, diethylene glycol monoethers, propylene glycol, etc.). Specific examples of these esters include dibutyl adipate, di(2-ethylhexyl) sebacate, di-n-hexyl fumarate, dioctyl sebacate, diisooctyl azelate, diisodecyl azelate, dioctyl phthalate, didecyl phthalate, dieicosyl sebacate, the 2-ethylhexyl diester of linoleic acid dimer, and the complex ester formed by reacting one mole of sebasic acid with two moles of tetraethylene glycol and two moles of 2-ethyl-hexanoic acid, and the like. A preferred type of oil from this class of synthetic oils is adipates of C₄ to C₁₂ alcohols.

Esters useful as synthetic lubricating oils also include those made from C₅ to C₁₂ monocarboxylic acids and polyols and polyol ethers such as neopentyl glycol, trimethylolpropane pentaerythritol, dipentaerythritol, tripentaerythritol, and the like.

Silicon-based oils (such as the polyalkyl-, polyaryl-, polyalkoxy-, or polyaryloxy-siloxane oils and silicate oils) comprise another useful class of synthetic lubricating oils. These oils include tetra-ethyl silicate, tetraisopropyl silicate, tetra-(2-ethylhexyl) silicate, tetra-(4-methyl-2-ethylhexyl) silicate, tetra-(p-tert-butylphenyl) silicate, hexa-(4-methyl-2-pentoxy)-disiloxane, poly(methyl)-siloxanes and poly(methylphenyl) siloxanes, and the like. Other synthetic lubricating oils include liquid esters of phosphorus-containing acids (e.g., tricresyl phosphate, trioctyl phosphate, and diethyl ester of decylphosphonic acid), polymeric tetra-hydrofurans, poly-α-olefins, and the like.

The lubricating oils may be derived from refined, rerefined oils, or mixtures thereof. Unrefined oils are obtained directly from a natural source or synthetic source (e.g., coal, shale, or tar sands bitumen) without further purification or treatment. Examples of unrefined oils include a shale oil obtained directly from a retorting operation, a petroleum oil obtained directly from distillation, or an ester oil obtained directly from an esterification process, each of which is then used without further treatment. Refined oils are similar to the unrefined oils except that refined oils have been treated in one or more purification steps to improve one or more properties. Suitable purification techniques include distillation, hydrotreating, dewaxing, solvent extraction, acid or base extraction, filtration, and percolation, all of which are known to those skilled in the art. Rerefined oils are obtained by treating used oils in processes similar to those used to obtain the refined oils. These rerefined oils are also known as reclaimed or reprocessed oils and are often additionally processed by techniques for removal of spent additives and oil breakdown products.

Another class of suitable lubricating oils are those basestocks produced from oligomerization of natural gas feed stocks or isomerization of waxes. These basestocks can be referred to in any number of ways but commonly they are known as Gas-to-Liquid (GTL) or Fischer-Tropsch base stocks.

When the lubricating oil is a mixture of natural and synthetic lubricating oils (i.e., partially synthetic), the choice of the partial synthetic oil components may widely vary, however, particularly useful combinations are comprised of mineral oils and poly-α-olefins (PAO), particularly oligomers of 1-decene.

The following examples are given as specific illustrations of the claimed invention. It should be understood, however, that the invention is not limited to the specific details set forth in the examples. All parts and percentages are by weight unless otherwise specified.

### Examples

A modification of the Ford MERCON® friction test (MERCON® Automatic Transmission Fluid Specification for Service, dated September 1, 1992. Section 3.8) was chosen to demonstrate the friction durability of the fluids of the invention. The Ford test stresses friction durability by using a low volume of fluid, and high test energy per cycle. Repeated dissipation of this high energy into this small volume of test fluid for 10,000 cycles is a strenuous evaluation of the fluid's ability to maintain constant frictional characteristics. This Ford test method was modified as shown below:

**Test as performed:**

| | |
|---|---|
| Friction material: | Borg Warner 6100 (not grooved) |
| Test temperature: | 115°C |
| Total test cycles: | 10,000 |
| Cycles per minute: | 3 |
| Total energy per cycle: | 20,400 J |
| Piston apply pressure: | 275 kPa |

**Static friction measurement:**

| | |
|---|---|
| Speed: | 4.37 rpm |
| Apply pressure: | 275 kPa |

Static friction: Measured after 2 sec of rotation

Since the principle role of the friction modifiers of the current invention is to reduce static friction, and maintain that level throughout the life of the fluid, the products of the invention were compared to the non-acylated versions in the SAE#2 friction test described above comparing stability of the static friction coefficient (Mu-s or µs).

Three test fluids were blended using exactly the same base lubricating oils, dispersants, anti-oxidants, and viscosity modifiers. The test blends contained the most preferred source of oil soluble phosphorus (Example G above), prepared as described in U.S. 5,314, 633. Into each fluid was added 3.0 mass percent of the friction modifier as follows:
Fluid A contained the product of Example B
Fluid B contained the product of Example C
Fluid C contained the product of Example D

The compositions of the test fluids and a summary of the test results are given in Table Ibelow.

As can be seen from Table 1, the normal friction modifier of Example B (Fluid A) has a decrease in static friction of 0.013 over the period of 500 to 10,000 cycles. The fluids containing the products of the invention, the products of Examples C and D exhibit lower changes in static friction : for Fluid B, a decrease of 0.002 and for Fluid C, a decrease of 0.003.

It is therefore clear that the acylation of the alkylene amine based friction modifiers has resulted in improved friction stability over the course of the test.

**Table 1**

| **TEST FORMULATIONS AND TEST RESULTS** | | | |
|---|---|---|---|
| COMPONENT | BLENDS | | |
| | 1* | 2 | 3* |
| Borated PIBSA/PAM Dispersant | 3.60 | 3.60 | 3.60 |
| Non-Borated PIBSA/PAM Dispersant | 1,50 | 1.50 | 1.50 |
| Alkylated Diphenyl Amine Anti-Oxidant | 0.75 | 0.75 | 0.75 |
| Hindered Phenol Anti-Oxidant | 0.25 | 0.25 | 0.25 |
| Alkyl Mercaptothiadiazole | 0.09 | 0.09 | 0.09 |
| Product of Example G | 0.40 | 0.40 | 0.40 |
| Product of Example A | 0.30 | 0.30 | 0.30 |
| Product of Example B | 3.30 | | |
| Product of Example C | - | 3.30 | - |
| Product of Example D | - | - | 3.30 |
| Thioalkyl ester | 0.10 | 0.10 | 0.10 |
| Long chain fatty acid | 0.10 | 0.10 | 0.10 |
| Long chain fatty amide | 0.10 | 0.10 | 0.10 |
| Calcium Sulfonate, 300 TBN | 0.20 | 0.20 | 0.20 |
| Sulfolane based seal swellant | 1.5 | 1.5 | 1.50 |
| Polymethacrylate Viscosity Modifier | 3.00 | 3.00 | 3.00 |
| Group III Basestock | 84.81 | 84.81 | 84.81 |
| | | | |
| Total | 100.00 | 100.00 | 100.00 |
| | | | |
| Static Friction Change 500 to 10,000 cycles | 0.013 | 0.002 | 0.003 |

| | | | |
|---|---|---|---|
| * examples not according to the invention | | | |

## Claims

1. A lubricating oil composition comprising a base lubricating oil, at least one oil soluble thioalkyl phosphite ester compound in an amount delivering from 5 to 5000 ppm of phosphorus into the oil and at least one polyalkylene polyamine-based friction modifier having the structure: in an amount of 0.1 to 10 weight percent in the composition.

2. The use of a composition according to claim 1 in a power transmission.

## Patentansprüche

1. Schmierölzusammensetzung, die Basisschmieröl, mindestens eine öllösliche Thioalkylphosphitesterverbindung, in einer Menge, die in dem Öl 5 bis 5.000 ppm Phosphor bereitstellt, und mindestens ein Reibungsmodifizierungsmittel auf Basis von Polyalkylpolyamin mit der Struktur: in einer Menge von 0.1 bis 10 Gew.-% in der Zusammensetzung umfasst.

2. Verwendung einer Zusammensetzung gemäß Anspruch 1 in einer Kraftübertragung.

## Revendications

1. Composition d'huile lubrifiante comprenant une huile lubrifiante de base, au moins un composé ester de thioalkylphosphite soluble dans l'huile en une quantité délivrant de 5 à 5000 ppm de phosphore dans l'huile et au moins un modificateur de frottement à base de polyalkylène-polyamine ayant la structure : en une quantité de 0,1 à 10 pour cent en poids dans la composition.

2. Utilisation d'une composition selon la revendication 1 dans une transmission de puissance.
